

## UNITED STATES PATENT OFFICE

2,533,096

## PRODUCTION OF IRON POWDER

Herschel H. Cudd and Emma Jean Freeman,  
East Point, Ga., assignors to International  
Minerals & Chemical Corporation, a corpora-  
tion of New York

No Drawing. Application August 17, 1945,  
Serial No. 611,260

8 Claims. (Cl. 204—10)

1

This invention relates to the production of relatively pure iron in small particles. Such a product is referred to in the trade as "iron powder," although it is not necessarily produced by mechanical comminution of larger particles. For most of the desired uses the configuration and porosity of the individual particles are significant. In general the more porous or dendritic the particle is, the better results can be obtained in the later fabrication of articles from it. These characteristics are not without limitation in that it is conceivable that it might be possible to get the particles too porous or too dendritic, but in the known processes, the common difficulty is the production of particles that do not have these characteristics to the extent desired for best results.

According to the invention, iron in finely divided form is precipitated electrolytically from an aqueous solution of an iron salt, for example a ferrous chloride or sulfate.

*Concentration*

In the case of the chloride it is possible to get satisfactory results when the concentration, expressed in terms of the percentage of weight of the tetrahydrate, is from below 10% to saturation at about 70%, the amount of ferrous ion in solution being, respectively, 2.8% and 19.7%. However, solutions having concentrations of about 25% to 35%, 7.0% and 9.9% ferrous ion respectively, apparently give best results under the conditions herein described.

*Temperature*

In the bath hereinafter described the quality of the deposit appears to be relatively independent of temperature over fairly wide limits. However, in order to produce a material of fine particle size it is advisable to employ relatively low temperatures, for example less than 40° C.

*Electrodes*

In the bath hereinafter described it is not necessary to rotate the electrode or employ mechanical means for removing the deposit from the electrode. The deposit is so lacking in adherence that a great deal of it falls off of its own accord and a very slight agitation or stirring will remove the rest. For instance, mere removal of the contents of the bath at a reasonably rapid rate will generate enough turbulence to wash the remaining deposit off the electrode.

2

*Current density*

Satisfactory operation is easily obtainable as low as 25 amperes per square foot if sufficient modifying agent is added to the bath. A material reduction in particle size results from using higher current densities, for example as high as 140 amperes per square foot. With suitably designed cells it is not difficult to deliver 140 amperes per square foot without excessive power loss.

*Modifying agent*

The modifying agents added to the bath to secure the unique fine grained dendritic deposit according to the invention include various materials which serve as foaming agents in iron salt solutions. A considerable variety of these agents have been tried and they all appear to be effective to some extent although some of them are materially better than others. Among the materials which have been used with appreciable advantage are the hydrophilic colloids such as saponins, peptones, gelatins, albumins, pectins and caseins.

Best results so far have been secured from saponin prepared from Chile soap bark, but substantially equal effectiveness has been secured with a saponin in the form of pure digitonin. The digitonin we have employed is a white crystalline substance which on acid hydrolysis splits into one mol of digitogenin, four mols of galactose and one mol of xylose. It is soluble in water and very soluble in methanol and hot ethanol. It has a specific rotation of —55° in methanol. Another identifying test is that, on the average, 1,000 milligrams will precipitate 330 milligrams of cholesterol in 100 cc. of 90% ethyl alcohol.

*Acidity*

Best results have been obtained so far when the pH is about 1.8 to 2.0 but a substantial variation from this figure does not materially impair the results. For example good results have been obtained with a pH of 1.0 to 3.0.

*Size control*

The grain size decreases rapidly with increase in the percentage of foaming agent in the bath. For instance, in one specific example, a bath containing 0.1% of saponin and operating at 26° C. gave the screen analysis in the middle column of the following table, while a bath otherwise identical except that it contained 0.3% of saponin and

3

operated at the same temperature gave the analysis in the right hand column:

| Mesh                    | 0.1% saponin |          | 0.3% saponin |          |
|-------------------------|--------------|----------|--------------|----------|
|                         | Per cent     | Per cent | Per cent     | Per cent |
| Does not pass 20.....   | 18.0         | .0       |              |          |
| Between 20 and 45.....  | 55.0         | 9.9      |              |          |
| Between 45 and 65.....  | 16.2         | 34.6     |              |          |
| Between 65 and 100..... | 5.6          | 19.8     |              |          |
| Passes 100.....         | 5.3          | 35.8     |              |          |

The screen analysis of the right hand column approximates the grain size and grain size distribution desirable for the fabrication of metal articles from the iron powder. It will be apparent that a very accurate control is thus secured which includes the desirable size range for the product. The percentage of modifying agent in the solution being electrolyzed may be varied from about 0.1 to about 0.6 per cent, the larger the percentage of modifying agent, the smaller the particle size of the iron powder which is formed.

#### Recovery from the bath

Separation of the precipitated metal from the liquid is not difficult, but obvious precautions need to be taken to guard against oxidation or even explosion. Especially in the finer grain sizes the product is decidedly pyrophoric and may ignite with destructive violence if dried and exposed to air. A satisfactory procedure is to filter and wash the residue first with ordinary water then with a .1% solution of ammonium carbonate or hydroxide, and finally with water which has been freshly boiled to eliminate dissolved oxygen. After this washing the product may be reduced to dryness in the absence of oxygen. If desired, the particle size may be further reduced by grinding under non-oxidizing conditions in any suitable mill. To obtain a very soft pure product, it may advantageously be annealed in hydrogen.

The process as described is of particular value for producing an iron powder in which the particles are of small size, and in a highly porous or dendritic condition. It may be used without grinding in the production of pressure-molded parts, particularly sintered parts.

Without further elaboration the foregoing will so fully explain the invention that others may adapt the same for use under various conditions of service.

What is claimed is:

1. The improvement in the art of producing iron powder, which comprises: electrolyzing an aqueous solution of an iron salt selected from the group consisting of ferrous chloride and ferrous sulfate, said solution being at a pH of between about 1.0 and 3.0 and containing at least about 2.8 per cent of ferrous ion, said solution also containing at least about 0.1 per cent of a hydrophilic colloid, which in said solution, will function as a foaming agent, the current density during electrolysis being between about 25 and 140 amperes per square foot.

2. The method of producing iron powder which is adapted for use in the fabrication of sintered parts, which comprises: preparing an aqueous solution of ferrous chloride which contains from about 7.0 to about 9.9 per cent ferrous ion and from about 0.1 to about 0.6 per cent of digitonin; adjusting the acidity of the solution to a pH of between about 1.8 and about 2.0; electrolyzing

4

the solution to deposit iron as a dendritic powder by employing a current density of from about 25 to about 140 amperes per square foot; and separating the iron powder from the solution, the size range of the dendritic iron particles being determined by the percentage of digitonin in the solution, the particle size decreasing with an increased concentration of digitonin.

3. The method of producing iron powder which comprises: preparing an aqueous electrolyte which contains at least about 2.8 per cent ferrous ion and at least about .1 per cent of a saponin, adjusting the acidity of the electrolyte to a pH of between about 1.0 and about 3.0; electrolyzing the electrolyte to deposit iron as a dendritic powder by employing a current density of from about 25 to about 140 amperes per square foot; and separating the iron powder from the electrolyte.

10 4. The method of producing iron powder which comprises: preparing an aqueous electrolyte which contains from about 7.0 to about 9.9 per cent ferrous ion and from about 0.1 to about 0.6 per cent of a saponin, adjusting the acidity of the 25 solution to a pH of between about 1.8 and about 2.0; electrolyzing the electrolyte to deposit iron as a dendritic powder by employing a current density of from about 25 to about 140 amperes per square foot; and separating the iron 30 powder from the electrolyte, the size range of the iron particles being determined by the percentage of saponin in the solution, the particle size decreasing with an increased concentration of saponin.

35 5. The method of producing iron powder which comprises: preparing an aqueous electrolyte which contains at least about 2.8 per cent ferrous ion and at least about .1 per cent of Chile-soap-bark saponin, adjusting the acidity of the 40 electrolyte to a pH of between about 1.0 and about 3.0; electrolyzing the electrolyte to deposit iron as a dendritic powder by employing a current density of from about 25 to about 140 amperes per square foot; and separating the iron 45 powder from the electrolyte.

6. The method of producing iron powder which comprises: preparing an aqueous electrolyte which contains from about 2.8 to about 19.7 per cent ferrous ion and from about 0.1 to about 0.6 per cent of Chile-soap-bark saponin, adjusting the acidity of the solution to a pH of between about 1.0 and about 3.0; electrolyzing the electrolyte to deposit iron as a dendritic powder by employing a current density of from about 25 55 to about 140 amperes per square foot; and separating the iron powder from the electrolyte, the size range of the iron particles being determined by the percentage of saponin in the solution, the particle size decreasing with an increased concentration of saponin.

7. The method of producing iron powder which comprises: preparing an aqueous electrolyte which contains from about 7.0 to 9.9 per cent ferrous ion, the salt supplying the ferrous ion 65 being selected from the group consisting of ferrous chloride and ferrous sulfate, and about 0.3 per cent of Chile-soap-bark saponin; adjusting the acidity of the solution to a pH of between about 1.8 and 2.0; electrolyzing the electrolyte 70 to deposit iron as a dendritic powder by employing a current density of from about 25 to 140 amperes per square foot; and separating the iron powder from the electrolyte.

8. The method of producing iron powder which 75 comprises preparing an aqueous electrolyte

which contains over about 2.8 per cent ferrous ion and over about .1 per cent of a digitonin, adjusting the acidity of the electrolyte to a pH of between about 1.0 and about 3.0; electrolyzing the electrolyte to deposit iron as a dendritic powder by employing a current density of from about 25 to about 140 amperes per square foot; and separating the iron powder from the electrolyte.

HERSCHEL H. CUDD.  
EMMA JEAN FREEMAN.

| Number       | Name          | Date          |
|--------------|---------------|---------------|
| 1,931,854    | Teats         | Oct. 24, 1933 |
| 2,157,699    | Hardy         | May 9, 1939   |
| 2,233,103    | Mantel        | Feb. 25, 1941 |
| 5 2,287,082  | Bauer         | June 23, 1942 |
| 2,389,180    | Brown         | Nov. 20, 1945 |
| 2,420,403    | Stoddard      | May 13, 1947  |
| 2,464,168    | Balke         | Mar. 8, 1949  |
| 2,464,889    | Pike et al.   | Mar. 22, 1949 |
| 10 2,480,156 | Matson et al. | Aug. 30, 1949 |

## FOREIGN PATENTS

| Number     | Country       | Date         |
|------------|---------------|--------------|
| 15 329,324 | Great Britain | May 14, 1930 |

## OTHER REFERENCES

|                                                                                     |
|-------------------------------------------------------------------------------------|
| Transactions of American Electrochemical Society, vol. 25 (1914), pages 529 to 532. |
| The Metal Industry, Oct. 7, 1938, page 350.                                         |

## UNITED STATES PATENTS

| Number    | Name   | Date          |    |
|-----------|--------|---------------|----|
| 949,004   | Ramage | Feb. 15, 1910 | 15 |
| 1,912,430 | Cain   | June 6, 1933  | 20 |

**Certificate of Correction**

December 5, 1950

**Patent No. 2,533,096**

**HERSCHEL H. CUDD ET AL.**

It is hereby certified that error appears in the printed specification of the above numbered patent requiring correction as follows:

Column 2, line 25, for "casiens" read *caseins*; column 4, line 75, after the word "comprises" insert a colon; column 5, line 5, for "deposite" read *deposit*; column 6, list of references cited, under the heading "OTHER REFERENCES" add the following—

*The Journal of the Iron and Steel Institute, vol. 109 (1924) No. 1, pages 409-414.*

and that the said Letters Patent should be read as corrected above, so that the same may conform to the record of the case in the Patent Office.

Signed and sealed this 13th day of March, A. D. 1951.

**[SEAL]**

**THOMAS F. MURPHY,  
Assistant Commissioner of Patents.**